

Oct. 26, 1937.

H. L. MUNROE

2,097,089

COATED FABRIC AND METHOD OF MAKING THE SAME

Filed July 8, 1936

*Fig. 1.*



*Fig. 2.*



*Fig. 3.*



*Fig. 4.*



*Inventor:*

*Howard L. Munroe,  
Dymer Booth Lorraine Miller Weidner  
Attns*

## UNITED STATES PATENT OFFICE

2,097,089

COATED FABRIC AND METHOD OF MAKING  
THE SAME

Howard L. Munroe, Malden, Mass.

Application July 8, 1936, Serial No. 89,519

4 Claims. (Cl. 91—68)

This invention relates to a leather-like coated fabric and the method of making the same. It contemplates a product comprising a textile fabric base or strain-resisting, flexible backing 5 bound or united to a facing layer of comminuted cork applied in such manner that a fabric is produced of light weight, substantial body, water and heat resisting properties, great flexibility and tensile strength and with a surface finish such that it is applicable to a wide variety of uses.

This application is a continuation in part of my prior co-pending application, Serial No. 691,013, filed September 26, 1933.

A cork coated fabric of the type hereinafter described may be employed, among other uses, as a vamp lining for shoes, for innersoles, as a substitute for leather in the manufacture of artificial leather and particularly imitation patent leather, either by the customary hand jpanning process or by a pyroxylin coating, and for numerous other purposes where lightness, body, flexibility and water resisting properties are desirable.

The invention will be best understood by reference to the following description of one or more specific embodiments thereof when taken in connection with the accompanying illustration, while its scope will be more particularly pointed out in the appended claims.

30 In the drawing:

Fig. 1 is a representation of the cork coated face of a fabric embodying one form of the invention;

Fig. 2 is a cross-sectional elevation, on a greatly exaggerated scale, of the fabric shown in Fig. 1;

Fig. 3 is a similar cross-sectional elevation showing the addition of a coating to provide an imitation patent leather;

Fig. 4 is a diagrammatic representation of a coating and drying machine which may be employed in carrying out the process; and

Fig. 5 is a diagrammatic representation of an apparatus employed for surfacing the cork.

The physical characteristics of the cork coated fabric may be best explained in connection with a description of one method employed in producing it.

The textile fabric for the base or backing of the product is selected according to the use to which the coated fabric is to be applied. For example, in the case of its use for shoe vamp linings, a white twill-weave cotton fabric may be employed, the weight of which, by way of example, may be one-half pound to the yard. If 55 the coated fabric is intended to be used for imita-

tion patent leather, to secure added flexibility a more finely finished and somewhat lighter weight of cotton twill may be employed, such as that known as sateen weave, this being dyed to a color corresponding to the patent leather finish.— 5 brown, for example, if a brown finish is to be applied, or black if a black finish is used.

The selected textile fabric, in the form of a continuous strip, has applied to one side thereof a plastic coating composed of a cellulose ester 10 binding solution which, for example, may consist of pyroxylin or cellulose acetate. On this there is then spread or distributed a quantity of comminuted or granular cork, the latter being caused to adhere to the coated side of the textile fabric. 15 The cork coated fabric then passes through a drying device, after which it is wound on a roll preparatory for the next operation.

An apparatus of the type diagrammatically shown in Fig. 4 may be employed for the coating 20 and drying operation. This comprises the supply roll 11 on which the fabric 13 is wound, the latter being then fed over guide rollers and under tension onto the coating table 15 where the plastic solution is applied to and spread across its surface. 25 The solution may be applied by hand or fed under suitable regulation from a supply chamber 17. The fabric is then fed beneath the doctor blade 19, passing thence, while still wet and sticky from the plastic coating, into the cork 30 box 21 which is kept filled with finely granulated cork. The fabric strip passes down through the mass of cork and thence upward and out of the same, accumulating on its coated tacky surface 35 a covering of the granulated cork particles. The loose particles of cork are removed from the under-surface of the fabric as it emerges from the cork box by a rotary brush 23. From the cork box the fabric passes into and through a 40 drying chamber 25 over guide rollers 27, describing looped paths between which are positioned steam drying pipes 29. The drying of the fabric may be further accelerated by the introduction into the drying room of hot air through the hot air pipes 31. The dried fabric on emerging from the drying room is wound up on the winding roll 33.

If a pyroxylin solution is employed, this may be composed of nitro cellulose and a suitable 50 solvent, with a small quantity of castor oil to give flexibility to the fabric. As an example of the solvent, it may comprise 25% of ethyl acetate, 25% of alcohol, and 50% of benzol, 24 ounces of nitrocellulose being added to each gal- 55

ion of the solvent and mixed into the form of a jelly.

As an example of cellulose acetate, if that be employed, the solvent may comprise 30% chemically pure acetone, 30% ethyl acetate, 20% "methyl cellosolve" (ethylene glycol monoethyl ether) and 20% of a plasticizer, such, for example, as that commonly known as M 17. To each gallon of solution there is added 32 ounces of cellulose acetate which is mixed into the form of a jelly.

The process is herein described as carried out through the use of pyroxylin but may be performed by the same steps when other cellulose ester solutions are made use of, as, for example, cellulose acetate.

The solution should be sufficiently thick and viscous to cause the ready adherence of the cork to the coated surface to provide a bond and anchorage for the cork coating and to bind and blend with the innermost cork granules when the fabric is subjected to the compression hereinafter described. The solution, however, should be sufficiently fluid to penetrate the fibers on the face of the textile fabric to be coated, but preferably without marked tendency to strike through the fabric and mar the original clean appearance of the uncoated face of the latter by evidences thereon either of the solution or the cork particles. This desired condition is promoted by slightly starching the fabric before being coated, to size the same.

I have found that any evidence of the discoloration referred to may be avoided by first sizing the fabric with a coating of pyroxylin solution and drying the same, as by such means as are indicated in Fig. 4, but without the intermediate step of applying the cork to the coated surface. The fabric, thus preliminarily coated with pyroxylin, if that be the case, is then passed through the operation just previously described, and in the apparatus represented in Fig. 4, that is to say, by applying a second coat of pyroxylin to the previously coated surface, followed by the addition thereto of the cork and the drying operation. This preliminary coating step I prefer to employ in connection with products where such discoloration may be a disadvantage. It may also be advantageously used for the purpose of imprinting a body to the underlying fabric backing, which is important in certain applications, such, for example, as where the product is used for vamp linings for shoes.

The cork coated fabric as it emerges from the drying room presents a rough, granular surface, the innermost cork granules being firmly united to the face of the textile fabric and the outermost particles less firmly united. Loose particles of cork may be removed from the surface by subsequently subjecting the fabric to the action of a suitable brushing machine before it is further worked upon.

The cork coated fabric is subsequently subjected to operations serving to impart solidity, firmness, and a finished surface to the cork.

For certain products a single coating of the cork will suffice. Preferably, however, to give the desired body to the cork covering, the fabric coated as previously described is next subjected to a second coating operation. That is to say, the winding roll 33 carrying the cork coated, dried and brushed fabric is transferred to the supply stand in place of the supply roll 11, and the cork coated fabric is again fed through the coating machine, cork box, drying room and brushing

machine, thereby superimposing on the face of the original cork coating another coating of pyroxylin, and on the top of the pyroxylin a second layer of granular cork, which latter becomes set and bonded to the under layers by the drying operation.

The fabric with the double layers of cork bound thereto is then subjected to a solidifying and firming action. A simple method of securing the desired result is to feed the double coated fabric between steam heated calendering rolls heated to a temperature just sufficient to very slightly soften the pyroxylin without disturbing the bond and adjusted to exert a substantial compression upon the coated fabric as it passes between them. Or, in place of heated calendering rolls, a friction calender may be used so adjusted as to generate a sufficient amount of heat to soften the pyroxylin. Cork is highly compressible and one result of the calendering and heating operation is to compact closely the granules of cork to cause the further spreading or penetration of the two layers or coatings of pyroxylin into the interstices between the particles or granules and the fibers thereof, thereby binding the cork particles into a more compact condition which they permanently retain. This imparts a relatively greater solidity, strength and permanency to the coating, the cork particles, and more particularly those in close proximity to the pyroxylin, being blended, as it were, into the pyroxylin binder. The calendering operation also imparts a smooth, even surface to the cork on the coated side of the fabric.

A calendering operation similar to the one described, to which the fabric is subjected after the application of the second coating of cork, may in many instances, depending on the use to which the product is to be put, be advantageously applied to the fabric after the application of the first coating of cork and before the application of the second cork coating. Such intermediate calendering tends further to compact the cork and improve its bond as well as the surface thereof.

The fabric with its solidified coating produced by any of the steps hereinbefore described and its calendered surface may then be subjected to a smoothing operation designed to remove any unevenness in the surface of the cork face due to irregularities in the distribution or thickness of the cork, or to other causes, and designed further to provide a soft surface finish by raising a fine nap on the face of the cork, which finish closely resembles the finish of suede leather in appearance and feel.

This operation may be performed by subjecting the cork face of the fabric to the carefully controlled and regulated abrading or buffing operation of the apparatus which is diagrammatically represented in Fig. 5. In this apparatus the fabric 13, with the coated face downward, is fed under tension over the plate 35, beneath the feed rollers 31 and between the buffering cylinder 39 and the guiding roll 41, the latter being susceptible of very fine adjustment in a vertical direction to secure a close, exact regulation of the space between the surface of the buffering cylinder and the guide roll. The buffering cylinder is suitably surfaced, as with fine sand paper or other abrading or buffering material, and is also so constructed that, besides being rotated at a high rate of speed, it has imparted to it a reciprocating axial movement, this insuring an evenly distributed buffering action over the cork.

surface without the production of scratches or other marring effects.

The buffing action carried out in the manner described produces a soft surface on the cork, characterized by the seemingly napped appearance of the cork face interspersed with occasional minute pores, closely resembling the surface appearance of suede leather.

The finished appearance of the fabric made by the use of the two cork coatings as described is illustrated in Figs. 1 and 2. Referring to Fig. 2, where an attempt has been made to represent a cross-section of the fabric on a greatly exaggerated scale, the textile backing is indicated at 43, this being firmly bonded to the adjacent pyroxylin coating at 45. The first or inner cork layer is represented at 47, the outer or surface cork layer at 49, and the intervening pyroxylin at 51. The inner cork layer 47 becomes more or less blended with the underlying pyroxylin 45 and the overlying pyroxylin 51, and the bottom of the outer cork layer becomes similarly more or less blended with the pyroxylin coating 51. The surface of the outer cork layer or coating will be free from any appearance of the pyroxylin, the cork layer thus completely covering and concealing the underlying cellulose ester binder.

The fabric thus produced has a substantial body or thickness for a given weight, this characteristic making it particularly available for the vamp lining of a shoe, since a single piece vamp lining cut from this fabric may be employed in substitution for the several pieces of fabric commonly required for that purpose and which comprise the fabric lining itself, a doubler to give body to the lining, and in many cases a rubberized backing cloth for the leather. The fabric herein described is also waterproof or water-resisting, heat insulating, of substantial tensile strength, capable of being stitched, and of a flexibility approximating that of the textile fabric forming the base or backing and substantially equal to that of leather of the same thickness.

These qualities make it available for a wide variety of uses. One use which may be referred to is as a base for imitation patent leather. An example of this is shown in Fig. 3, where the cork coated fabric substantially similar to that previously described has had applied to the outer cork surface a facing of pyroxylin 53 imparting to it a patent leather finish.

In the manufacture of the imitation patent leather, and in some cases in the manufacture of the fabric for other purposes, it may be desirable to reverse the order of the buffing and the calendering operations, the cork coated fabric being first buffed and then calendered instead of being first calendered and then buffed. In the case of imitation patent leather this provides a smooth, even surface for the finally finished cork coating to which the outer pyroxylin coating for the patent leather may be applied with better effect and appearance.

The pyroxylin facing 53 may be built up by passing the cork coated fabric through a coating machine and applying the pyroxylin to the cork coated surface in the usual manner, drying the coating and repeating the operation a sufficient number of times to get the necessary depth and finish to the facing, the pyroxylin solution applied in the successive coats being varied in respect to thinness to secure the necessary glossy surface finish. The pyroxylin solution, with the addition of a pigment giving the necessary color,

may be made up of nitro-cellulose, with a sufficient solvent of the character previously described, preferably using also a small quantity of castor oil mixed with the solution.

Due to the peculiar characteristics of the cork coated fabric, it may be successfully and practically employed as a body for the production of imitation patent leather produced by the japaning process instead of the machine coating method last described. That process, as is well known, is carried out by manually applying to the leather,—or in this case the cork coated fabric,—by brushing or rubbing into the surface thereof a succession of coats comprising principally linseed oil mixed with a suitable pigment, the material being dried or baked between successive coats.

The cork coated fabric makes a particularly useful imitation patent leather, since it provides a body beneath the surface finish similar to that of leather, with a flexibility adequate to counteract any tendency to crack the surface. Furthermore, it is water resisting, in which respect it is superior to leather for use in footwear where the penetration of moisture and its absorption from within the shoe tends to the deterioration and the cracking of the patent leather surface finish.

The cork coated fabric is particularly useful in the manufacture of imitation grained or embossed leathers. These have been usually made by applying pyroxylin coats directly to the face of a textile fabric and then embossing the coated face of the fabric under heavy pressure. In this method it is difficult to eliminate the evidence of the weave in the cloth except through the use of an excessive number of coatings. The cork coating on the described fabric, presenting a smooth, uniform surface, offers no such objection and being highly compressible facilitates the production of the embossing design.

It is preferred to dye the comminuted cork prior to its incorporation in the fabric when the product is intended for uses wherein it would be noticeable and the natural cork color might be considered objectionable, for example, when the product simulates patent leather.

While I have herein shown for purposes of illustration one specific embodiment of the coated fabric comprising the invention and have described one method by which it may be produced, extensive deviations may be made in the method of production and in the product, all without departing from the spirit of the invention.

I claim:

1. As a new article of manufacture, a flexible patent leather-like fabric comprising a sheet of woven textile material, a sizing of cellulose ester selected from the group consisting of cellulose acetate and cellulose nitrate applied directly to the material and having a penetrating anchorage in the body thereof, a like cellulose ester binder overlying said sizing, a layer of comminuted cork completely covering and concealing the binder firmly united thereto and compressed therein, said cork layer having a smooth leather-like surface and a yielding base, said fabric further having an outer glossy patent leather-like facing comprising a plurality of coats of nitrocellulose covering the smooth surface of the cork, the coated fabric possessing flexibility comparable to the flexibility of the original woven textile material.

2. The method of making a cork coated fabric to imitate leather while maintaining substantially the flexibility of the fabric which comprises sizing a woven textile fabric base with a cellulose

ester solution selected from the group consisting of cellulose acetate and cellulose nitrate to provide a coating having a penetrating anchorage in the fabric base protecting said base against 5 discoloration, drying said protective coating, applying a coating of like cellulose ester binder directly to said dried protective coating, immediately applying a relatively thick layer of com- 10 minuted cork thereto completely covering and concealing said binder before the latter dries, quickly and thoroughly drying said binder under heat, and calendering the fabric after the cork coating and binder have become dried and set.

3. The method of making a cork coated fabric 15 to imitate patent leather while maintaining substantially the flexibility of the fabric base which comprises sizing a woven textile fabric base with a cellulose ester solution selected from the group consisting of cellulose acetate and cellulose ni- 20 trate to provide a coating having a penetrating anchorage in the fabric base protecting said base against discoloration, drying said protective coating, applying a coating of like cellulose ester binder directly to said dried protective coating, 25 immediately applying a relatively thick layer of comminuted cork thereto completely covering and concealing said binder before the latter dries,

quickly and thoroughly drying said binder under heat, calendering the fabric after the cork coating and binder have become dried and set, and applying a plurality of coats of patent leather-like facing to said calendered surface, and thoroughly drying said coats between successive applications. 5

4. The method of making a cork coated fabric to imitate leather while maintaining substantially the flexibility of the fabric base which comprises sizing a woven textile fabric base with a cellulose ester solution selected from the group consisting of cellulose acetate and cellulose nitrate to provide a coating having a penetrating anchorage in the fabric base protecting said base against 15 discoloration, drying said protective coating, applying a coating of like cellulose ester binder directly to said dried protective coating, immediately applying a relatively thick layer of com- 20 minuted cork thereto completely covering and concealing said binder before the latter dries, quickly and thoroughly drying said binder under heat, and calendering the fabric after the cork coating and binder have become dried and set under heat and pressure to slightly soften the 25 binder and compress the cork layer therein.

HOWARD L. MUNROE.